

## UNITED STATES PATENT OFFICE

ROYER LUCKENBACH, OF BROOKLYN, NEW YORK

## PROCESS OF CONCENTRATING ORES

No Drawing.

Application filed October 9, 1925. Serial No. 61,588.

The invention relates to the concentration of ores by the froth flotation process, and has for its object to provide a cheap but powerful froth flotation oil having as its base a petroleum residue which will select or gather the mineral content of the ore.

I have discovered that a heavy petroleum residuum or still bottoms has exceptional mineral selecting properties, surpassing coal tars heretofore used in the flotation of ores when properly diluted or thinned and combined with a strong frothing agent. I have found this mineral selecting quality to be strongest in residuum petroleum oil, more so than in any of the fractions from it. The frother I have found to be very effective in combination with the petroleum is wood or pine pitch diluted in a suitable solvent as kerosene oil, or an alkaline solution of pine pitch, carbon disulphide, alcohol and water, which is the subject matter of a recent application, Serial No. 33,506, May 28th, 1925. Other light petroleum distillates are equally as effective as kerosene as a pitch solvent, but the use of carbon disulphide with pine pitch and alcohol is particularly beneficial in treatment of highly basic ores, owing to its elimination of iron from the concentrates when combined with caustic soda or potash, and water as a dilutent. This combination forms the preferred frother, and being also a strong selector the mixture of it with the petroleum oil, also a strong mineral selector, produces a powerful flotation of oil very suitable for practically all the principal ores, and its action is still further increased when an alkaline circuit is used in the flotation machines. With an alkaline circuit the amount of oil used is greatly reduced.

Although the pitch xanthate solution as above is very effective as a frother, small amounts of additional frothing agents can be used, as pine oil, sulphonated castor oil, cottonseed foots, pine creosote, pine tar and rosin, on special ores as carbonates of copper, zinc and lead, also oxides and silicates of these metals upon which sulphonated castor oil and cottonseed foots are very effective when combined with the petroleum prepared as specified.

This class of ores, of which there are vast deposits in South America and Africa, have been most difficult to recover by any known oils heretofore. Among other oils I have found to be very effective with wood pitch to form a strong frother with petroleum, is Scotch blast furnace oil, or the ketones, as acetone, ketone residue, etc.

As a dilutent of the petroleum residuum I make use of kerosene oil or any cheap distillate, together with pine pitch and carbon disulphide to form a thin solution, or can use a solution of kerosene and pine creosote or pine tar. The use of the pine element is to give the dilutent a frothing quality that greatly adds to the efficiency of the petroleum oil when the regular frother is added.

Having described my invention, what I claim as new and desire to secure by Letters Patent is:

1. The process of concentrating ores by flotation, which comprises adding to the mineral pulp an emulsified product of petroleum oil and a pitch and xanthate frother, agitating the pulp under alkaline conditions to form a froth and separating the froth from the pulp.

2. The process of concentrating ores by flotation, which comprises adding to the mineral pulp an alkaline solution of a resinous product, carbon disulphide, alcohol and petroleum oil, agitating the pulp to form a froth and separating the froth from the pulp.

3. The process of concentrating ores by flotation, which comprises adding to the mineral pulp a diluted petroleum residue, an alkaline solution of wood pitch, carbon disulphide, alcohol and water, agitating the pulp to form a froth and separating the froth from the pulp.

4. The process of concentrating ores by flotation, which comprises adding to the mineral pulp an emulsion of 50 to 70% of a heavy petroleum residuum, 10 to 15% of a petroleum dilutent for thinning the residuum, and 10 to 30% of a frother of wood pitch and xanthate as described, agitating the pulp under alkaline conditions to form a froth and separating the froth from the pulp.

5. The process of concentrating ores by

flotation, which comprises adding to the mineral pulp an emulsion of petroleum oil, a xanthate and a frother, agitating the pulp under alkaline conditions to form a froth and separating the froth from the pulp.

5 6. The improvement in the concentration of minerals by flotation which comprises subjecting the mineral in the form of a pulp to a flotation operation under alkaline condition in the presence of xanthate, a petroleum and sulphonated castor oil.

10 Signed at New York city in the county of New York and State of New York this 8th day of October A. D. 1925.

15 ROYER LUCKENBACH.

20

25

30

35

40

45

50

55

60

65